

# UNITED STATES PATENT OFFICE.

JOHN T. H. DEMPSTER, OF SCHENECTADY, NEW YORK, ASSIGNOR TO GENERAL ELECTRIC COMPANY, A CORPORATION OF NEW YORK.

## PROCESS OF MAKING ALLOYS.

No. 926,980.

Specification of Letters Patent.

Patented July 6, 1909.

Application filed March 28, 1908. Serial No. 423,907.

To all whom it may concern:

Be it known that I, JOHN T. H. DEMPSTER, a citizen of the United States, residing at Schenectady, in the county of Schenectady 5 and State of New York, have invented certain new and useful Improvements in Processes of Making Alloys, of which the following is a specification.

This invention relates to alloys of various 10 metals and has for its object the production of alloys by a process which is simple and at the same time lends itself to the formation of an alloy in which the composition is accurately and definitely known.

15 In my previous patent No. 901,428, I have described and claimed a resistance conductor which has valuable properties adapting it to a variety of uses. This alloy is heat-refractory to an extraordinary degree. It 20 does not easily oxidize when subjected to a prolonged red heat in the atmosphere. It is acid-proof and has high electrical resistivity adapting it for electric heating and rheostat work. The slight oxidation which the wire 25 undergoes from prolonged red heat goes on slowly and the oxid is coherent and does not materially change its conductivity. The composition which I have found very successful contains approximately

30 62 parts nickel (by weight)  
20 parts iron "  
13 parts chromium "  
5 parts manganese "

35 In the melting of this alloy it was found that carbon must be excluded from the mixture since otherwise the alloy became hard and brittle. It was found moreover that nickel is high in carbon and that it is therefore necessary to purify the nickel in making up the alloy. Graphite crucibles cannot be used because of the fact that the metals of the alloy will take up carbon. Clay-lined crucibles serve the purpose excepting for the 45 fact that the manganese attacks the clay and exposes the graphite. The following process has been found to operate satisfactorily. In the bottom of a clay-lined graphite crucible is placed an oxid to serve as a decarbonizer.

50 This oxid may be hematite ( $Fe_2O_3$ ). It is found that about eight pounds of this oxid is necessary for one hundred pounds of alloy. Nickel is then charged into the crucible with a small quantity of silica and cryolite as flux,

and when the nickel is melted the heat is run 55 up to promote a vigorous reaction between the oxid and the carbon. This reaction is shown by the gas bubbles igniting above the slag and burning with a blue flame. When the metal quiets down, the carbon being 60 eliminated, the iron is added and after this is melted the chromium is added. While the mixture is in a molten condition, care being taken not to excessively heat the metal and burn the lining, the manganese is added in 65 suitable quantities. The mixture is then quickly poured before the manganese attacks the clay lining.

By this process I am able to practically eliminate the carbon from the mixture and 70 obtain an accurately proportioned alloy in a simple manner.

While I have described my invention in connection with specific metals mixed in certain portions as well as steps of the process 75 taken in a certain way, it should be understood that I do not limit my invention thereto except in so far as it is limited by the scope of the claims annexed hereto.

What I claim as new and desire to secure 80 by Letters Patent of the United States, is,

1. The process of producing alloys which consists in melting a quantity of nickel with a de-carbonizing agent in a clay lined crucible to reduce the carbon, adding iron and 85 chromium in suitable proportions, then adding manganese and pouring the mixture before the manganese attacks the clay lining.

2. The process of producing alloys which consists in first de-carbonizing a quantity of 90 nickel in a clay-lined crucible, successively adding other metals in suitable proportions including manganese and then pouring the mixture before the manganese attacks the clay lining.

95 3. The process of producing alloys which consists in first de-carbonizing a quantity of nickel in a clay-lined crucible, successively adding chromium and manganese in suitable proportions and then pouring the mixture 100 before the manganese attacks the clay lining.

In witness whereof, I have hereunto set my hand this 26th day of March, 1908.

JOHN T. H. DEMPSTER.

Witnesses:

P. H. SMITH,  
T. P. THOMPSON.